# EUROPEAN PATENT SPECIFICATION

(11) **EP 3 136 819 B1**
(45) Date of publication and mention of the grant of the patent: **06.05.2020**
(21) Application number: 15782910.2
(22) Date of filing: 27.04.2015
(51) Int. Cl.: H05B 3/02, H05B 3/12, H05B 3/14, H05B 3/18, H05B 3/06, H05B 3/48

(54) **HEATER AND IGNITION DEVICE**
HEIZER UND ZÜNDUNGSVORRICHTUNG
DISPOSITIF DE CHAUFFAGE ET DISPOSITIF D'ALLUMAGE

(30) Priority: 25.04.2014 JP 2014090911
(43) Date of publication of application: 01.03.2017
(73) Proprietor: Kyocera Corporation, Kyoto-shi, Kyoto 612-8501 (JP)
(72) Inventor: NAGAMORI, Hirokazu, Kyoto-shi Kyoto 612-8501 (JP)
(74) Representative: Viering, Jentschura & Partner mbB Patent- und Rechtsanwälte
(86) International application number: PCT/JP2015/062651
(87) International publication number: WO 2015/163483

(56) References cited:
- EP-A1- 1 696 704
- EP-A1- 1 711 034
- EP-A1- 2 996 438
- EP-A2- 0 914 021
- WO-A1-2013/047849
- JP-A- H01 272 078
- JP-A- H11 126 675
- JP-A- 2001 244 053
- JP-B2- 2 537 271
- JP-B2- 2 828 575
- JP-B2- 3 121 860
- JP-B2- 3 924 193
- JP-B2- 4 183 186
- JP-B2- 5 357 628
- JP-U- H0 429 192

## Description

### Technical Field

The present invention relates to a heater and an ignition device.

### Background Art

A heater (ceramic heater) in which a heat-generating body is disposed in a ceramic body is known as an example of a heater for use in a gas stove, an on-vehicle heating device, a kerosene fan heater, a glow plug of an automobile engine, or the like. Patent Document 1 discloses an example of a ceramic heater.

Japanese Unexamined Patent Application Publication No. 2000-156275 (hereinafter referred to as Patent Document 1) discloses a ceramic heater including a ceramic structure, a heat-generating resistor embedded in the ceramic structure, and feeder lines that are connected to the heat-generating resistor and extend to a surface of the ceramic structure.

The ceramic heater described in Patent Document 1 has a risk that cracks will be formed in the feeder lines when the ceramic heater is repeatedly used in a high-temperature environment. When, in particular, cracks are formed in portions of the feeder lines exposed at the surface of the ceramic structure, the outside air may flow into the feeder lines. Therefore, the resistance of the feeder lines may change due to a reaction between the feeder lines and the outside air, and abnormal local heat generation may occur. Thus, it is difficult to increase the long-term reliability when the ceramic heater is repeatedly used in a high-temperature environment.

EP 2 996 438 A1, a document which falls under Art. 54(3) EPC, discloses that a ceramic heater comprises a ceramic structure, a heat-generating resistor embedded in the ceramic structure, and a feeder line embedded in the ceramic structure so as to be connected, at one end thereof, to the heat-generating resistor (cf. Abstract). This document further discloses that the feeder line is made of metal and that metal grains of a center region of the feeder line are greater in grain size than metal grains of an outer periphery region of the feeder line.

EP 1 696 704 A1 discloses that a ceramic heater comprises a ceramic body, a heat generating resistor buried in the ceramic body, an electrode pad that is electrically connected to the heat generating resistor and is formed on the surface of the ceramic body and a lead member bonded onto the electrode pad (cf. Abstract).

WO 2013/047849 A1 discloses that a heater comprises an insulating base made of ceramic, and an electrically conductive line embedded in the insulating base, wherein the electrically conductive line contains electrically conductive grains and ceramic grains, and the ceramic grains in the electrically conductive line have a smaller average grain size than the ceramic grains in the insulating base (cf. Abstract).

### Summary of Invention

The present invention provides a heater according to claim 1. Further embodiments of the present invention are described in the dependent claims. A heater includes a ceramic multilayer body including a plurality of ceramic layers that are stacked together; a heat-generating resistor having a belt shape, the heat-generating resistor being disposed between the ceramic layers and arranged, and including both ends that are at a side surface of the ceramic multilayer body; and conductive layers having a belt shape, disposed between the ceramic layers and stacked on both end portions of the heat-generating resistor in such a manner that one end of each conductive layer is at the side surface. Each conductive layer includes a first conductive layer that extends to the side surface and a second conductive layer that is adjacent to the first conductive layer, each of the first conductive layer and the second conductive layer being formed of a plurality of grains, the grains of the first conductive layer having an average grain diameter smaller than an average grain diameter of the grains of the second conductive layer.

### Brief Description of Drawings

Fig. 1 is a longitudinal sectional view of a heater.
Fig. 2 is a cross-sectional view of the heater illustrated in Fig. 1 taken along line A-A'.
Fig. 3 is a cross-sectional view of the heater illustrated in Fig. 1 taken along line B-B'.
Fig. 4 is a cross-sectional view of a modification of the heater.
Fig. 5 is a perspective view of an ignition device including the heater illustrated in Fig. 1.

### Description of Embodiments

A heater 10 will be described with reference to the drawings.

As illustrated in Figs. 1 to 3, the heater 10 includes a ceramic multilayer body 1 including a plurality of ceramic layers 11 that are stacked together, a heat-generating resistor 2 provided between the adjacent ceramic layers 11, and conductive layers 3 stacked on the heat-generating resistor 2. The heater 10 may be used in, for example, a glow plug of an automobile engine or a gas stove.

The ceramic multilayer body 1 is a member in which the heat-generating resistor 2 and the conductive layers 3 are embedded. The durabilities of the heat-generating resistor 2 and the conductive layers 3 can be increased by placing the heat-generating resistor 2 and the conductive layers 3 in the ceramic multilayer body 1. The ceramic multilayer body 1 is, for example, a rod-shaped or plate-shaped member.

The ceramic multilayer body 1 is made of an electrically insulative ceramic, such as an insulating ceramic, a nitride ceramic, or a carbide ceramic. More specifically, the ceramic multilayer body 1 is made of, for example, an alumina ceramic, a silicon nitride ceramic, an aluminum nitride ceramic, or a silicon carbide ceramic.

The ceramic multilayer body 1 made of a silicon nitride ceramic may be obtained by the following method. For example, silicon nitride, which is the main component, is mixed with 5 to 15 mass% of rare earth oxide, such as Y₂O₃, Yb₂O₃, or Er₂O₃, which functions as a sintering additive; 0.5 to 5 mass% of Al₂O₃; and SiO₂, the amount of which is adjusted so that the amount of SiO₂ in the sintered body is 1.5 to 5 mass%. The thus-obtained material is formed in a predetermined shape, and is then fired at a temperature of 1650°C to 1780°C. Thus, the ceramic multilayer body 1 made of a silicon nitride ceramic is obtained. Hot press firing, for example, may be performed in the firing process.

When the ceramic multilayer body 1 is rod-shaped, more specifically, rectangular-prism-shaped, the length of the ceramic multilayer body 1 is set to, for example, 20 to 100 mm. The cross-sectional shape of the ceramic multilayer body 1 is set to, for example, a rectangle having a thickness of 1 to 6 mm and a width of 2 to 40 mm.

The heat-generating resistor 2 is a layer-shaped member that generates heat when a voltage is applied thereto. The heat-generating resistor 2 is disposed between the adjacent ceramic layers 11. When a voltage is applied to the heat-generating resistor 2, a current flows through the heat-generating resistor 2, and the heat-generating resistor 2 generates heat. The generated heat is transferred through the ceramic multilayer body 1, so that the temperature of the surface of the ceramic multilayer body 1 increases. The heat is transferred from the surface of the ceramic multilayer body 1 to an object to be heated, thereby providing the function of the heater 10. The object to be heated that receives the heat from the surface of the ceramic multilayer body 1 is, for example, diesel oil to be supplied to an automobile diesel engine.

The heat-generating resistor 2 is arranged in such a manner that both ends thereof are at a side surface of the ceramic multilayer body 1 near the rear end of the ceramic multilayer body 1. The heat-generating resistor 2 has, for example, a bent shape in longitudinal cross section (cross section parallel to the length direction of the heat-generating resistor 2). More specifically, the heat-generating resistor 2 includes two linear portions that are arranged next to each other and a connecting portion that has substantially semicircular or substantially semielliptical inner and outer peripheries and that is bent so as to connect the two linear portions. The heat-generating resistor 2 is bent at a location near the front end of the ceramic multilayer body 1. The total length of the heat-generating resistor 2 is, for example, 35 to 100 mm.

The heat-generating resistor 2 is designed so as to generate a large amount of heat in a region near the front end of the ceramic multilayer body 1. More specifically, the conductive layers 3 are stacked on both end portions of the heat-generating resistor 2 in a region near the rear end of the ceramic multilayer body 1. Accordingly, a current flows through both the heat-generating resistor 2 and the conductive layers 3 in the region near the rear end of the ceramic multilayer body 1. As a result, the amount of heat generated by the heat-generating resistor 2 is small in the region near the rear end of the ceramic multilayer body 1. In contrast, the current flows only through the heat-generating resistor 2 in the region near the front end of the ceramic multilayer body 1. As a result, the amount of heat generated by the heat-generating resistor 2 is large in the region near the front end of the ceramic multilayer body 1.

The heat-generating resistor 2 is made of, for example, a material having a carbide, nitride, silicide, etc., of tungsten (W), molybdenum (Mo), titanium (Ti), etc., as the main component. When the ceramic multilayer body 1 is made of a silicon nitride ceramic, the heat-generating resistor 2 is preferably made of a material having tungsten carbide as the main component. In this case, the coefficient of thermal expansion of the ceramic multilayer body 1 and that of the heat-generating resistor 2 can be made close to each other.

The conductive layers 3 are members for adjusting the amount of heat generated by the heat-generating resistor 2 in the region near the rear end of the ceramic multilayer body 1, that is, in the region around the portions of the side surface of the ceramic multilayer body 1 to which the heat-generating resistor 2 extends. In Fig. 1, the conductive layers 3 are shown by the broken lines. In Fig. 1, the broken lines that show the conductive layers 3 and the solid lines that show the heat-generating resistor 2 are shifted from each other to improve visibility. However, in practice, the conductive layers 3 and the heat-generating resistor 2 have substantially the same width, and are stacked together so as to be aligned with each other in the width direction. As illustrated in Figs. 2 and 3, the conductive layers 3 are stacked on both end portions of the heat-generating resistor 2 in the space between the ceramic layers 11, and are arranged such that one end of each conductive layer 3 is at the side surface of the ceramic multilayer body 1. By covering both end portions of the heat-generating resistor 2, which are to be connected to an external circuit, with the conductive layers 3, the amount of heat generated in the region near the rear end of the ceramic multilayer body 1 can be reduced. Accordingly, the connection reliability between the external circuit and the heater 10 can be increased.

Each conductive layer 3 includes a first conductive layer 31 that extends to the side surface of the ceramic multilayer body 1 and a second conductive layer 32 that is adjacent to the first conductive layer 31. The first conductive layer 31 and the second conductive layer 32 are each formed of a plurality of grains. The average grain diameter of the grains of the first conductive layer 31 is smaller than that of the grains of the second conductive layer 32. Since the first conductive layer 31, which is located closer to the outside, is formed of grains having a small average grain diameter, the density of the first conductive layer 31 can be increased. As a result, the voidage of the first conductive layer 31 is reduced, and the risk that the outside air will flow into each conductive layer 3 can be reduced.

Since not only the conductive layers 3 but also the heat-generating resistor 2 extends to the side surface of the ceramic multilayer body 1, portions that extend to the side surface have a two-layer structure. Therefore, even when cracks are formed either in the conductive layers 3 or in the heat-generating resistor 2, the risk that the cracks will extend into the other of the conductive layers 3 and the heat-generating resistor 2 can be reduced.

Since the second conductive layer 32 is formed of grains having a large average grain diameter, the number of grain boundaries of the grains of the second conductive layers 32 can be reduced. Therefore, the resistance of the second conductive layer 32 can be reduced. Accordingly, unnecessary heat generation by each conductive layer 3 can be suppressed.

As a result, the long-term reliability of the heater 10 when used in a heat cycle is increased.

More specifically, for example, in the case where conductive layers having a constant average grain diameter in each portion thereof are provided, unlike the above-described heater 10, the following problem arises. That is, when the average grain diameter of the conductive layers is simply reduced, even though the risk that the outside air will flow into the conductive layers can be reduced, since the resistance of the conductive layers increases, unnecessary heat generation by the conductive layers occurs. Conversely, when the average grain diameter of the conductive layers is simply increased, even though unnecessarily heat generation by the conductive layers can be suppressed, the outside air easily flows into the conductive layers. In contrast, by making the average grain diameter of the grains of the first conductive layer 31 smaller than that of the grains of the second conductive layer 32 as in the above-described heater 10, the risk that the outside air will enter each conductive layer 3 can be reduced and unnecessary heat generation by each conductive layer 3 can be suppressed.

In addition, as illustrated in Fig. 2, the first conductive layer 31 and the second conductive layer 32 preferably partially overlap. In such a case, unlike the case in which the first conductive layer 31 and the second conductive layer 32 do not overlap, each conductive layer 3 can be formed so as to have a coefficient of thermal expansion that changes gradually in the length direction thereof. As a result, the possibility that cracks will be formed in the conductive layers 3 in a heat cycle can be reduced.

Preferably, the first conductive layer 31 is located between the second conductive layer 32 and the heat-generating resistor 2, and, in a region in which the first conductive layer 31 is located between the second conductive layer 32 and the heat-generating resistor 2, the first conductive layer 31 has a thickness that decreases toward the other end thereof. In such a case, each conductive layer 3 can be formed so as to have a coefficient of thermal expansion that changes smoothly. As a result, the possibility that cracks will be formed in the conductive layers 3 in a heat cycle can be further reduced.

In the above-described heater 10, each conductive layer 3 includes only the first conductive layer 31 and the second conductive layer 32. However, each conductive layer 3 is not limited to this, and may further include a portion other than the first conductive layer 31 and the second conductive layer 32. For example, as illustrated in Fig. 4, each conductive layer 3 may include, in addition to the first conductive layer 31 and the second conductive layer 32, a third conductive layer 33. The third conductive layer 33 is adjacent to the second conductive layer 32 at a side opposite to the side adjacent to the first conductive layer 31.

There is no particular limitation regarding the layer used as the third conductive layer 33. For example, the third conductive layer 33 may be formed of grains having an average grain diameter smaller than that of the grains of the second conductive layer 32. In such a case, the number of crystal grain boundaries of the grains of the third conductive layer 33 can be increased. Accordingly, the resistance of the third conductive layer 33 can be set to a value higher than that of the second conductive layer 32. Therefore, the amount of heat generated by the heat-generating resistor 2 can be changed gradually. Accordingly, the surface of the heater 10 can be heated in such a manner that the temperature thereof changes gradually. As a result, the risk that a large local thermal stress will be generated in the ceramic multilayer body 1 can be reduced.

The first to third conductive layers 31 to 33 are made of, for example, a highly heat-resistant metal material, such as molybdenum (Mo), tungsten (W), or rhenium (Re). MoSi₂, WSi₂, etc., are preferably mixed in the material to make the coefficient of thermal expansion close to that of the ceramic multilayer body 1. The length of a portion of the first conductive layer 31 that extends in the length direction of the heat-generating resistor 2 is set to about 2 to 10 mm. The thickness of the first conductive layer 31 is set to about 5 to 30 µm. The length of a portion of the second conductive layer 32 that extends in the length direction of the heat-generating resistor 2 is set to about 5 to 20 mm. The thickness of the second conductive layer 32 is set to about 25 to 75 µm. In the case where the first conductive layer 31 and the second conductive layer 32 overlap, the length of the overlapping region is set to, for example, about 500 µm.

The grain diameters of the first conductive layer 31 and the second conductive layer 32 can be adjusted as follows. In the case where the first conductive layer 31 and the second conductive layer 32 are both made of W, the grain diameters of the first conductive layer 31 and the second conductive layer 32 can be adjusted by changing the particle diameter of W powder, which is the starting material. For example, the average grain diameter of the W powder used to form the first conductive layer 31 may be set to 0.2 µm, and the average grain diameter of the W powder used to form the second conductive layer 32 may be set to 1.2 µm. In this case, the average grain diameter of the first conductive layer 31 can be set to 0.2 to 2 µm, and the average grain diameter of the second conductive layer 32 can be set to 1.2 to 12 µm.

In particular, the average grain diameter of the first conductive layer 31 is preferably less than 1 µm. In such a case, entrance of the outside air into the first conductive layer 31 through the spaces between the grains can be suppressed, and therefore the risk that the outside air will flow into the first conductive layer 31 can be reduced. The voidage of the first conductive layer is preferably less than 20%. In such a case, entrance of the outside air into the first conductive layer 31 can be suppressed.

The average grain diameter of each conductive layer 3 can be determined by, for example, the following method. That is, the heater 10 is cut along a plane that passes through the conductive layer 3 and that is perpendicular to the conductive layer 3 by using a diamond cutter. Then, the cut surface is ground by using diamond powder. After that, the first conductive layer 31 and the second conductive layer 32 are observed by using a scanning electron microscope or metallographic microscope. More specifically, five arbitrary straight lines are drawn on the image obtained by the scanning electron microscope or metallographic microscope. Then, the average of the lengths of portions of the five straight lines, each portion passing through ten grains, is determined. The average grain diameter is determined by dividing the average by ten, which is the number of grains. The average grain diameter may instead be calculated by using an image analyzing device (LUZEX-FS produced by Nireco Corporation). This image analyzing device can also be used to measure the voidage of the first conductive layer 31.

The heater 10 is used in, for example, an ignition device 100 illustrated in Fig. 5. The ignition device 100 includes the heater 10 and a channel 20 through which fuel gas is supplied to the heater 10. The channel 20 includes, for example, a gas valve 21 and a gas flow pipe 22 having ejection holes 23. The gas valve 21 has a function of controlling the flow rate of the fuel gas. The fuel gas supplied from the gas valve 21 is, for example, natural gas or propane gas. The gas flow pipe 22 ejects the fuel gas, which is supplied from the gas valve 21, toward the heater 10 through the ejection holes 23. The ejected fuel gas can be ignited by heating the fuel gas with the heater 10. The ignition device 100, which includes the heater 10 having improved long-term reliability, has increased fuel-gas ignition stability.

### Reference Signs List

- 1: ceramic multilayer body
- 11: ceramic layer
- 2: heat-generating resistor
- 3: conductive layer
- 31: first conductive layer
- 32: second conductive layer
- 10: heater
- 20: channel
- 21: gas valve
- 22: gas flow pipe
- 23: ejection hole
- 100: ignition device

## Claims

1. A heater (10) comprising:
a ceramic multilayer body (1) comprising a plurality of ceramic layers (11) that are stacked together;
a heat-generating resistor (2) having a belt shape and comprising two ends, the heat-generating resistor (2) being disposed between the ceramic layers (11) and arranged such that both ends are at a side surface of the ceramic multilayer body (1) ; and
conductive layers (3) having a belt shape, disposed between the ceramic layers (11) and stacked on both end portions of the heat-generating resistor (2) in such a manner that one end of each conductive layer is at the side surface;
wherein each conductive layer comprises a first conductive layer (31) that extends to the side surface and a second conductive layer (32) that is adjacent to the first conductive layer (31), each of the first conductive layer (31) and the second conductive layer (32) being formed of a plurality of grains, the grains of the first conductive layer (31) having an average grain diameter smaller than an average grain diameter of the grains of the second conductive layer (32).

2. The heater (10) according to Claim 1, wherein the first conductive layer (31) and the second conductive layer (32) partially overlap.

3. The heater (10) according to Claim 2, wherein, in a region in which the first conductive layer (31) and the second conductive layer (32) overlap, the first conductive layer (31) is located between the second conductive layer (32) and the heat-generating resistor (2), and
wherein, in a region in which the first conductive layer (31) is located between the second conductive layer (32) and the heat-generating resistor (2), the first conductive layer (31) has a thickness that decreases toward the other end of the first conductive layer (31).

4. The heater (10) according to any one of Claims 1 to 3, wherein the grains of the first conductive layer (31) have an average grain diameter of 0.2 to 2 µm, and the grains of the second conductive layer (32) have an average grain diameter of 1.2 to 12 µm.

5. The heater (10) according to any one of Claims 1 to 4, wherein the first conductive layer (31) has a voidage of less than 20%.

6. An ignition device (100) comprising:
the heater (10) according to any one of Claims 1 to 5; and
a channel (20) through which fuel gas flows to the ceramic multilayer body (1) included in the heater (10).

## Patentansprüche

1. Heizvorrichtung (10), aufweisend:
einen Keramikmehrschichtkörper (1), der eine Mehrzahl von Keramikschichten (11) aufweist, die übereinandergestapelt sind,
einen wärmeerzeugenden Widerstand (2), der eine Bandform hat und zwei Enden aufweist, wobei der wärmeerzeugende Widerstand (2) zwischen den Keramikschichten (11) angeordnet ist und derart angeordnet ist, dass sich beide Enden an einer Seitenfläche des Keramikmehrschichtkörpers (1) befinden, und
leitfähige Schichten (3), die eine Bandform haben, die zwischen den Keramikschichten (11) angeordnet und derart auf beide Endabschnitte des wärmeerzeugenden Widerstands (2) gestapelt sind, dass ein Ende jeder leitfähigen Schicht an der Seitenfläche liegt,
wobei jede leitfähige Schicht eine erste leitfähige Schicht (31), die sich zu der Seitenfläche erstreckt, und eine zweite leitfähige Schicht (32), die benachbart zu der ersten leitfähigen Schicht (31) ist, aufweist, wobei jede von der ersten leitfähigen Schicht (31) und der zweiten leitfähigen Schicht (32) aus einer Mehrzahl von Körnern gebildet ist, wobei die Körner der ersten leitfähigen Schicht (31) einen durchschnittlichen Korndurchmesser haben, der kleiner als ein durchschnittlicher Korndurchmesser der Körner der zweiten leitfähigen Schicht (32) ist.

2. Heizvorrichtung (10) gemäß Anspruch 1, wobei die erste leitfähige Schicht (31) und die zweite leitfähige Schicht (32) teilweise überlappt sind.

3. Heizvorrichtung (10) gemäß Anspruch 2, wobei in einem Bereich, in dem die erste leitfähige Schicht (31) und die zweite leitfähige Schicht (32) überlappt sind, die erste leitfähige Schicht (31) sich zwischen der zweiten leitfähigen Schicht (32) und dem wärmeerzeugenden Widerstand (2) befindet, und
wobei in einem Bereich, in dem sich die erste leitfähige Schicht (31) zwischen der zweiten leitfähigen Schicht (32) und dem wärmeerzeugenden Widerstand (2) befindet, die erste leitfähige Schicht (31) eine Dicke hat, die in Richtung zu dem anderen Ende der ersten leitfähigen Schicht (31) kleiner wird.

4. Heizvorrichtung (10) gemäß irgendeinem der Ansprüche 1 bis 3, wobei die Körner der ersten leitfähigen Schicht (31) einen durchschnittlichen Korndurchmesser von 0,2 bis 2 µm haben und die Körner der zweiten leitfähigen Schicht (32) einen durchschnittlichen Korndurchmesser von 1,2 bis 12 µm haben.

5. Heizvorrichtung (10) gemäß irgendeinem der Ansprüche 1 bis 4, wobei die erste leitfähige Schicht (31) einen Hohlraumanteil von weniger als 20% hat.

6. Zündvorrichtung (100), aufweisend:
die Heizvorrichtung (10) gemäß irgendeinem der Ansprüche 1 bis 5 und
einen Kanal (20), durch den Brenngas zu dem in der Heizvorrichtung (10) enthaltenen Keramikmehrschichtkörper (1) strömt.

## Revendications

1. Dispositif de chauffage (10), comprenant :
un corps céramique multicouche (1) comprenant une pluralité de couches céramiques (11) qui sont empilées les unes sur les autres ;
une résistance génératrice de chaleur (2) présentant une forme de ruban et comprenant deux extrémités, la résistance génératrice de chaleur (2) étant disposée entre les couches céramiques (11) et agencée de telle sorte que les deux extrémités se trouvent sur une surface latérale du corps céramique multicouche (1) ; et
des couches conductrices (3) en forme de ruban, disposées entre les couches céramiques (11) et empilées sur les deux parties d'extrémité de la résistance génératrice de chaleur (2) de telle sorte qu'une extrémité de chaque couche conductrice se trouve sur la surface latérale ;
dans lequel chaque couche conductrice comprend une première couche conductrice (31) qui s'étend jusqu'à la surface latérale et une deuxième couche conductrice (32) qui est adjacente à la première couche conductrice (31), chacune de la première couche conductrice (31) et de la deuxième couche conductrice (32) étant formée d'une pluralité de grains, les grains de la première couche conductrice (31) ayant un diamètre moyen de grain inférieur à un diamètre moyen de grain des grains de la deuxième couche conductrice (32) .

2. Dispositif de chauffage (10) selon la revendication 1, dans lequel la première couche conductrice (31) et la deuxième couche conductrice (32) se chevauchent partiellement.

3. Dispositif de chauffage (10) selon la revendication 2, dans lequel, dans une région dans laquelle la première couche conductrice (31) et la deuxième couche conductrice (32) se chevauchent, la première couche conductrice (31) est située entre la deuxième couche conductrice (32) et la résistance génératrice de chaleur (2), et
dans lequel, dans une région dans laquelle la première couche conductrice (31) est située entre la deuxième couche conductrice (32) et la résistance génératrice de chaleur (2), la première couche conductrice (31) présente une épaisseur qui diminue vers l'autre extrémité de la première couche conductrice (31).

4. Dispositif de chauffage (10) selon l'une quelconque des revendications 1 à 3, dans lequel les grains de la première couche conductrice (31) ont un diamètre moyen de grain de 0,2 à 2 µm, et les grains de la deuxième couche conductrice (32) ont un diamètre moyen de grain de 1,2 à 12 µm.

5. Dispositif de chauffage (10) selon l'une quelconque des revendications 1 à 4, dans lequel la première couche conductrice (31) présente un pourcentage de vide de moins de 20%.

6. Dispositif d'allumage (100), comprenant :
le dispositif de chauffage (10) selon l'une quelconque des revendications 1 à 5 ; et
un canal (20) au travers duquel du gaz combustible s'écoule vers le corps céramique multicouche (1) compris dans le dispositif de chauffage (10).
